

A. JEDEL.

PYROTECHNIC DEVICE.

APPLICATION FILED AUG. 8, 1913.

1,094,999.

Patented Apr. 28, 1914.

Fig. 1.



Fig. 5.



Fig. 2.



Fig. 4.



Fig. 6.



Fig. 3.



Fig. 7.



<sup>Inventor</sup>  
Aaron Jedel

Witnesses

Geo. Ackman Jr.  
Milton Martin

By Victor J. Evans

Attorney

# UNITED STATES PATENT OFFICE.

AARON JEDEL, OF NEW YORK, N. Y.

## PYROTECHNIC DEVICE.

1,094,999.

Specification of Letters Patent. Patented Apr. 28, 1914.

Application filed August 8, 1913. Serial No. 783,812.

To all whom it may concern:

Be it known that I, AARON JEDEL, a citizen of the United States, residing at New York, in the county of New York and State 5 of New York, have invented new and useful Improvements in Pyrotechnic Devices, of which the following is a specification.

The present invention relates to improvements in pyrotechnic devices, and has for 10 its object the production of devices or "eggs" for the production of "Pharaoh's snakes" so called, as well as the process of producing the same, and the composition of matter of which these are composed.

15 In the production of "Pharaoh's snakes" as ordinarily carried out, prior to my invention, it has been the practice to use mercuric sulfocyanid or thiocyanate,  $Hg(SCN)_2$ , the particles of which are bound together by the 20 addition of a small amount of glue or other adhesive. The slurry of this material, glue, and water, is run into small molds in which the solid material separates out, and after drying in the molds, more or less thoroughly, the molded pieces (usually cone shaped) are removed from the molds and packaged for the market. These are ordinarily called "snake eggs." These molded pieces (snake eggs) as made heretofore, are 25 very easily broken by handling, having very little strength, and if placed one dozen in a box, as is usually done, they will generally crumble more or less, by rubbing, one against another. They cannot withstand, 30 ordinarily such pressure as would normally be exerted by pinching the same between the thumb and fingers, but would be mostly broken up by such treatment.

In preparing my articles, I preferably 35 proceed as follows: A mixture of, for example, mercuric sulfocyanid, 90 parts by weight, talc (powdered), 6 parts by weight, precipitated chalk, 4 parts by weight, (which proportions may be varied, if desired) is made, preferably in any approved 40 form of mixing device, in which the materials come into contact with the air. The sulfocyanid being hygroscopic absorbs some water from the air, sufficient to make the 45 mass granulate more or less, but not sufficient to produce a wet appearing, or muddy mass, but on the contrary the mass appears to be dry, and somewhat granular. This is then fed to molds in which the mixture is 50 55 molded, under considerable pressure, into

"eggs" of the desired shape and size, to produce a "snake" or other similarly formed object.

The "eggs" produced according to my process are very much harder than those 60 made by the prior processes. They cannot be crushed between the fingers, and in packages do not break or grind each other up to any appreciable extent, during such handling as is common. Packages of these may 65 be carried for some time in the pocket, without this inconvenience and in ordinary shipment it is not necessary, or even advisable to wrap each in tissue paper to prevent breaking.

70 In the accompanying drawing, forming a part of this specification; I have given, by way of illustration, several shapes which I find to give particularly striking results.

In said drawings, Figures 1, 2, 3 and 4 75 represent front elevations of four different forms of "snake eggs" made in accordance with my invention, and Figs. 5, 6 and 7 represent side or end elevations of three different forms which may be used.

80 The invention herein is not limited to these shapes, since other shapes may be used, if desired.

It will be noted that in Figs. 1, 2, 4, 6 and 7, are shown shapes which have projections 85 or "legs"  $\alpha$  on their lower surfaces. These legs, I have found to have a special function in this art, not merely as a support, but to keep the bulk of the material up a short distance from the supporting surface on 90 which they are placed during the burning operation, in order to allow the entire mass of material to be readily consumed, and also these legs themselves burn and produce legs or tails on the finished "snake," to make 95 the same have a rather striking appearance. One leg only may be provided, near one end of the base, or near the middle, which will raise nearly all the bottom surface of the "egg" from the surface on which the 100 "egg" is burned.

By suitably shaping the articles or "eggs" I can produce shapes somewhat resembling horses, crocodiles, and others. The "snakes" or other shapes produced by 105 burning these articles, have a somewhat different appearance from those produced from the "eggs" previously known, in that they have a darker color, a sort of yellowish brown, with a coppery tint, and quite a bri- 110

lant surface, which has a rather scaly appearance, much more so than the snakes produced from the "eggs" previously known. These differences may be due to the differences in the composition used, or to the fact that they are more compressed, or partly due to both these reasons, I am not prepared to say which.

10 In place of the talc and chalk, suitable equivalents may of course be used.

If desired, I may add to the composition above stated, materials for producing special effects, such as special colors, hissing sounds, peculiar odors, etc., without departing from the spirit of my invention.

15 The term "egg" as used in the appended claims, is intended to refer to combustible pyrotechnic devices of the kind referred to in this specification.

20 What I claim is:—

1. A pyrotechnic egg having a hardness sufficient to make it practically impossible to crush the same between the fingers, said egg being composed of a mixture of materials including mercuric sulfocyanid, and an inert, non-combustible, inorganic material.

25 2. As an article of manufacture, a pyrotechnic composed of a mixture including mercuric sulfocyanid, chalk and talc.

30 3. As an article of manufacture, a pyrotechnic composed of a mixture including mercuric sulfocyanid, chalk and talc, the two latter, in combined amount representing only a minor proportion of the entire product.

35 4. As an article of manufacture, a pyrotechnic composed of a mixture including mercuric sulfocyanid, chalk and talc, the sulfocyanid being present as about 90% of the entire product.

40 5. An article of manufacture comprising a pyrotechnic egg, composed of a mixture containing mercuric sulfocyanid, 90%; powdered talc, 6%; and chalk 4%.

45 6. An article of manufacture comprising a pyrotechnic egg, composed of a mixture containing mercuric sulfocyanid, 90%;

powdered talc, 6%; and chalk 4%, said pyrotechnic being provided with legs.

7. A pyrotechnic egg composed of a mixture including mercuric sulfocyanid, chalk and talc having a hardness sufficient to make it practically impossible to crush the same between the fingers.

8. An irregularly surfaced pyrotechnic egg provided with a leg composed of mercuric sulfocyanid, 90%; talc, 6%; and chalk 4%, approximately.

9. A method of making pyrotechnic eggs, which comprises compressing, into a mold of suitable form, a mixture of materials including mercuric sulfocyanid, and an inert, non-combustible, inorganic material, such as will form a firm coherent product having a degree of hardness sufficient to render it practically impossible to crush said eggs, by such pressure as can ordinarily be exerted between the fingers.

10. A method of making pyrotechnic eggs which comprises compressing a mixture comprising mercuric sulfocyanid, talc, and chalk, into molds of appropriate form and applying sufficient pressure to the mixture in the molds, to produce an "egg" having sufficient strength to prevent crushing by such an amount of pressure as can ordinarily be applied by pinching between the fingers.

11. A method of making pyrotechnic eggs which comprises compressing a mixture comprising mercuric sulfocyanid, talc and chalk, in the proportions of about 90:6:4; into molds of appropriate form and applying sufficient pressure to the mixture in the molds, to produce an "egg" having sufficient strength to prevent crushing by such an amount of pressure as can ordinarily be applied by pinching between the fingers.

In testimony whereof I affix my signature in presence of two witnesses.

AARON JEDEL.

Witnesses:

FANNIE JEDEL,  
MATHILDA JEDEL.

Copies of this patent may be obtained for five cents each, by addressing the "Commissioner of Patents, Washington, D. C."